

## UNITED STATES PATENT OFFICE.

MENDEL PIANKO, OF CHICAGO, ILLINOIS.

## ANTIFRICTION BELT DRESSING.

No Drawing.

Application filed October 6, 1921. Serial No. 505,955.

To all whom it may concern:

Be it known that I, MENDEL PIANKO, a citizen of the United States, residing at Chicago, in the county of Cook and State of Illinois, have invented a new and useful Antifriction Belt Dressing, of which the following is a specification.

This invention relates to a composition of matter for use as a belt dressing to prevent 10 a belt from slipping upon its pulleys.

Another object is to provide a dressing which will act as a preservative for the belt and at the same time insure a positive grip by the belt on a pulley so that no matter 15 how loose the belt may be it will pull to its full capacity.

A further object is to provide a dressing which is clean, will not soil the hands or pulleys, and will keep the belt elastic.

Another object is to provide a dressing which when applied will cause the belt to run smoothly and free from noise.

The invention consists of the following ingredients substantially in the proportions stated, to wit:

|                                          |                    |
|------------------------------------------|--------------------|
| Celluloid waste or gun or soluble cotton | 16 oz.             |
| Alcohol (ethyl or methyl)                | $\frac{2}{3}$ gal. |
| Ethyl (or methyl) acetate                | $\frac{1}{3}$ gal. |

The first mentioned ingredient is combined with the mixture of alcohol and acetate in the proportions of one gallon of the mixture to 16 ounces of the celluloid waste

or soluble cotton. This solid base of waste or cotton will be dissolved and form pyroxylin. To each gallon of pyroxylin there is added  $\frac{1}{3}$  gallon of castor oil which step completes the process. The product produced in the manner described can be applied to a belt with a brush and will impart to the belt a slightly sticky surface which will grip the pulley tightly under all conditions and prevent the belt from slipping. It is to be understood that in the preparation of the composition of matter the use of either celluloid waste or gun or soluble cotton makes no change in the nature of the product and either ingredient can be considered the equivalent of the other. The same 50 remarks apply to the use of either acetate described.

What is claimed is:—

A composition of matter for use as a belt dressing to prevent slipping, consisting of 55 a solution of 16 oz. of soluble cotton in a mixture of  $\frac{2}{3}$  gal. of alcohol and  $\frac{1}{3}$  gal. of ethyl acetate, there being added  $\frac{1}{3}$  gal. of castor oil to a gallon of the solution, the resultant product, when applied to a surface and dried, having a slightly sticky surface. 60

In testimony that I claim the foregoing as my own, I have hereto affixed my signature in the presence of a witness.

MENDEL PIANKO.

Witness:

Ivy E. SIMPSON.